

No. 873,512.

PATENTED DEC. 10, 1907.

C. DAVIS.

FACE HARDENED STEEL PLATE.

APPLICATION FILED APR. 23, 1902.

Fig. 1.



Fig. 2.



Inventor  
Cleveland Davis.

Witnesses

Geo. H. Payne  
Almon A. Bateman

By  
William & Fisher,  
Attorneys

# UNITED STATES PATENT OFFICE.

CLELAND DAVIS, OF THE UNITED STATES NAVY, ASSIGNOR, BY MESNE ASSIGNMENTS, TO CARNEGIE STEEL COMPANY, OF PITTSBURG, PENNSYLVANIA, A CORPORATION OF NEW JERSEY.

## FACE-HARDENED STEEL PLATE.

No. 873,512.

Specification of Letters Patent.

Patented Dec. 10, 1907.

Original application filed April 10, 1901, Serial No. 55,124. Divided and this application filed April 23, 1902. Serial No. 104,379.

To all whom it may concern:

Be it known that I, CLELAND DAVIS, lieutenant, United States Navy, a citizen of the United States, stationed at Washington, in the District of Columbia, have invented certain new and useful Improvements in Face-Hardened Steel Plates, (Case E;) and I do hereby declare the following to be a full, clear, and exact description of the invention, such as will enable others skilled in the art to which it appertains to make and use the same.

My invention relates to the manufacture of a face hardened plate of steel, which is uniformly impregnated with carbon to a prescribed depth, and in which the carbon shades off decrementally, or in a gradually decreasing manner, below said depth, the percentage of carbon in that portion of the plate so impregnated being greater than the normal content of the body of the plate.

In my invention, the main objects to be obtained are first, to be able to regulate the depth of carbonization and of chill so as to preserve the most effective proportion between the hard face and the tough back; and second, at the same time to preserve the integral character of the metal throughout.

If the plate is heated by an electric furnace to any desired depth to a molten point or to one approaching fluidity, the back being kept comparatively cool, carbon can be introduced in the desired quantity and will be absorbed instantly or in a very short time. This carbon will be disseminated uniformly throughout the molten portion, and will shade away behind that portion into the body of the plate.

In all the processes of cementation hitherto employed, the shading off of carbon begins from the surface or immediately below it.

The accompanying drawings show the electric furnace described in my application, Serial Number 55,124, filed April 10, 1901, of which this is a division.

These drawings show one form of furnace suitable for the hardening of a plate according to my invention.

The same parts are indicated by the same letters in both the views.

Figure 1 represents a section through a furnace constructed for carbonizing armor plate, the section of the cover being shown along the line 1—1 of Fig. 2, and Fig. 2 rep-

resents an inverted plan view of the detachable air tight cover to go over the side of the plate that is to be heated.

A represents the masonry, preferably fire-brick, having the plate a, twyers a', and asbestos and fire clay backing a<sup>2</sup> let inside the same.

B represents the armor plate supported on I-beams C, which are insulated as at c. The entire plate should be insulated in this or any other convenient way.

D represents a removable cover which may be removed as by means of the cable E passing over the pulley F, or in any other convenient way. This cover makes an air tight joint over the side of the plate to be treated. The said cover is packed with asbestos, or fire clay, or similar material G, in which a plurality of electrodes H are held, and these electrodes are connected with the source of electricity by suitable conductors indicated diagrammatically at I. The circuit to the source of electricity is completed by means of the contacts K and the conductors L.

The contacts K may be placed at suitable points on the sides or bottom of the plate. A layer of powdered carbon M is interposed between the cover D and the face of the plate to be heated. Air, either hot or cold, may be blown through the twyers a' from any suitable air blast, not shown, and thus lower the temperature of the under side of the plate, while the upper side of the plate is being heated, or other means may be employed to keep the back of the plate cool, if preferred.

In practice the plate is put in position, a measured quantity of powdered or granular carbon M is spread over the surface to be treated, the cover D is lowered in place and the joints made tight, and the necessary electric current is turned on. This speedily raises the temperature of the carbon M and the upper part of the plate, until the latter reaches almost, if not quite, the fusing point, and the layers of carbon will be absorbed into the plate. In the meantime the lower part of the plate may be kept comparatively cool, by means of an air blast through the twyers a'. If the electric current be kept on until all the carbon M has disappeared, then it will be known that this has been carried into the body of the plate, and in this way a measured degree of carburization may be obtained. Moreover, by varying the current 105 along the line 1—1 of Fig. 2, and Fig. 2 rep-

and the time of its application, the carbon may be carried through into the plate, causing the cementation to be deeper than with the processes now in use.

- 5 A direct current would, I believe, be preferable to an alternating current, as the tendency of the carbon would be to follow the current. If desired, a single electrode might cover the entire mass of carbon M, or a single 10 carbon electrode might be used, covering the entire face of the plate to be treated, or the electrodes H might be differently grouped, and the current passed through them *seriatim*, or in groups, or the pulverized carbon M 15 might be done away with, and the carbon supplied direct from the carbon electrodes, all of which, and any other grouping of electrodes I intend to include within the scope of my claims.
- 20 Instead of having the circuit closed, I may establish an arc between the electrodes and the face of the plate to be treated, when disintegration of the electrodes will supply the carbon.
- 25 No hard and fast rule can be laid down as to the treatment of any particular class of plates, as the treatment would differ for different grades of steel, and for different sizes of plates, etc., but the electrical characteristics once being established, it is evident that 30 conditions can be reproduced with great accuracy by use of the volt meter and ammeter, and by regulating the amount of carbon to be introduced into the plate. It will be evident that this method of treatment may be 35 used with any plate or body of steel in which it is desired to surface harden.
- While I have described this invention as applied to the treatment of armor plate for 40 the purpose of face hardening the same, it will be obvious that the same is applicable to the cementation or hardening of steel plates

or bodies wherever it is desired to surface harden. It is obvious that both faces of the plate, or the entire surface of the body, may 45 be hardened if desired.

By the word "integral" in the claims, I intend to distinguish my product from one formed from two or more plates, making up 50 the compound plate.

Having thus described my invention, what I claim and desire to secure by Letters Patent of the United States, is:

1. An integral mass of steel the face of which is uniformly impregnated with absorbed carbon to a prescribed depth, the carbon decrementally shading off below that depth, the percentage of the carbon in the portion of the plate so impregnated being greater than the normal content of the body 60 of the plate substantially as described.

2. A hard faced armor plate composed of an integral mass of steel having one face impregnated with absorbed carbon uniformly to a prescribed depth, and the carbon shading off decrementally below that depth, the percentage of carbon in the portion of the plate so impregnated being greater than the normal content of the body of the plate substantially as described.

3. An integral steel plate having a surface portion or stratum of determinable depth containing a substantially uniform content of carbon which is higher than the normal content of the plate body, and an underlying portion or stratum in which the carbon content shades off decrementally into the body of the plate; substantially as described.

In testimony whereof, I affix my signature, in presence of two witnesses.

CLELAND DAVIS.

Witnesses:

CLARENCE A. BATEMAN,  
FRED W. ENGLERT.